

## UNITED STATES PATENT OFFICE

ROGER W. CUTLER, OF NEEDHAM, AND JOSEPH R. COOLIDGE, 3d, OF BROOKLINE, MASSACHUSETTS, ASSIGNEES TO MONTAN, INC., OF BOSTON, MASSACHUSETTS, A CORPORATION OF MASSACHUSETTS

## FIBER BOARD AND PROCESS OF MANUFACTURING FIBER BOARD

No Drawing.

Application filed May 27, 1927. Serial No. 194,852.

This invention relates to fiber board, wall board, and like products which are composed chiefly or entirely of unvulcanized fiber.

It is an important object of this invention so to improve the characteristics of the less expensive grades of fiber board and similar materials that their serviceability and range of usefulness will be greatly increased, and to make them suitable not only for many uses for which only the better grades of fiber board can now be used, but also to adapt them for some purposes to which it is impractical to apply the more expensive grades of fiber board.

15 The best grades of fiber board or fiber products are of the so-called "vulcanized" variety, and this grade of material is very hard, dense, and compact. It is a very stable product and is much used for electrical insulation and for mechanical purposes, where it is subjected to severe wear. The less expensive grades of fiber board and fiber articles are compressed and consolidated but are not vulcanized, and they are much softer, more porous, less resistant to moisture, and warp badly when exposed to moisture. When wet for long periods of time they show considerable tendency to disintegrate. While these materials are used as insulators for some purposes, 20 as for example in enclosed switches, their uses for this purpose are very limited, chiefly because they absorb moisture so readily that their dielectric strength is extremely variable. They withstand mechanical abrasion very poorly, and this fact also limits their range of usefulness.

Usually these grades of fiber board or fibrous bodies are composed chiefly of wood pulp, although they may also be made of other fibers of a woody nature, as for example, the fiber obtained from bagasse, corn stocks or grasses; but they often contain also a substantial percentage of rag stock or fiber made from rope or twine waste. The composition of those qualities of fiber board with which this invention is particularly concerned therefore varies considerably with the grade and price.

45 The products of this character which are used as wall boards are usually of a rela-

tively soft character, they have considerable affinity for moisture which often produces buckling or warping, and those of the very porous character usually are also highly inflammable.

We have discovered that the characteristic of all of these fiber boards or fiber bodies can be improved very materially by impregnating them with Montan wax. This is a mineral wax which usually is imported into this country but is readily obtainable in large quantities and at a moderate expense under the name above given. The melting point of this wax varies somewhat with different grades but usually is in the neighborhood of 180° F., and it has the peculiar property of remaining very hard and brittle as its temperature is raised until the melting point is almost reached, when it passes very rapidly from a solid to a liquid state. One grade or variation of this wax is known commercially as romalin wax and is also readily obtainable on the market although not so well known as Montan wax.

The method used in impregnating fiber board with Montan wax necessarily will vary somewhat with the characteristics of the material under treatment and the results desired. In treating the softer and more porous grades of fiber board or fiber bodies, such, as for example, as wall boards made chiefly from bagasse fiber, or the like, entirely satisfactory results can be produced simply by soaking the fiber board in a bath of the melted wax, the bath preferably being maintained at a temperature of somewhere in the neighborhood of 225° F. At this temperature the wax is absorbed very readily by the fiber board, and after only a relatively few moments of immersion, unless the material is uncommonly thick, it may be removed and allowed to drip.

In treating molded or compressed fiber bodies, or the better grades of unvulcanized fiber board, it is preferable to force the waxy material into the microscopic pores and cells of the fiber board under considerable pressure. For this purpose the fiber board or fiber articles may be placed in a cylinder or container capable of withstanding high pres-

sures and submerged in the melted wax, air then being pumped into the cylinder until the desired degree of pressure is produced. Assuming that the material under treatment is fiber board sheets of approximately one-quarter inch thickness, a suitable impregnation may be obtained by maintaining the material under a pressure of from 100 to 125 pounds for a period of one hour, the temperature of the wax being from, say, 225° to 250° F. The pressure, time, and temperature may all be varied, however, if desired, and as above indicated the exact procedure necessarily will depend upon the nature of the material under treatment and local conditions. A higher temperature facilitates impregnation, and the penetration of the wax also may be improved in treating difficult grades of material by using a small percentage, say 10%, of some liquid which is readily miscible with, or acts as a solvent for, the wax, such for example, as kerosene, benzol, carbon tetrachloride, or the like. When the treatment has been continued for the desired length of time, the pressure is relieved, and the material is withdrawn and allowed to drain and cool, whereupon the wax hardens or solidifies.

The methods above described produce a high concentration of the wax in the fiber board and greatly increase its weight. If for any reason such an increase in weight is not desired, the fiber board may be placed in the cylinder preparatory to impregnation and subjected to a preliminary air pressure which will substantially fill the microscopic pores and cells in the stock before the melted wax is admitted to the cylinder and allowed to submerge the fiber board. This pressure is maintained while the fiber board is being immersed in the wax, and the pressure then is increased so as to force the wax into the pores and cells of the fibrous body. Later when the impregnation has been completed and the external pressure is relieved, the air held in the pores and cells of the material expands and expels or ejects part of the wax so that the total quantity of wax ultimately retained by the material is reduced.

Fiber board or other fiber bodies which have been impregnated with Montan wax in the manner above described have characteristics and properties which present marked contrast to the untreated materials. The treated stock is harder, more dense and stable. It appears to be entirely unaffected by exposure to moisture and may even be submerged in water for long periods without undergoing material change. Its insulating properties are immensely improved and because of its greatly increased resistance to the effects of moisture, it can be used for insulation in a great variety of locations where the untreated material would be totally unfit for use. For example, the treated stock can be

successfully used in the insulation of the live rails of traction systems and for a variety of purposes where it is exposed to the weather and where the untreated material would certainly fail. This impregnated fiber product also is highly resistant to the attacks of most acids and will successfully withstand their action for periods of time far in excess of those required to destroy untreated fiber parts. In this respect the impregnated fiber is even superior to vulcanized fiber. Since the impregnated fiber board is substantially unaffected by moisture it does not shrink, swell or warp when exposed to moisture, and this fact also permits its use for many purposes where the untreated material cannot be used successfully. Wall boards impregnated in this manner are improved very greatly both because they will not shrink, swell or warp with changes in humidity, and also because the board is made much stronger, stiffer, and more stable. The bonding of the fibers together with the wax in addition to the natural mechanical bonding of the fibers with each other, forms a product which is much superior mechanically to the untreated stock.

The waxy material itself is not readily inflammable so that the porous grades of wall board which are highly combustible are made much less inflammable by the treatment.

In case it is desired to mold the fiber board, or to work it into complicated or unusual shapes, it is preferable in some instances to perform the molding or shaping operation after the board has been impregnated and before it has cooled. For example, in forming curved sheets or flat sheets which are to be used for switch panels, or the like, and where it is desired to have the surfaces substantially true, the impregnated sheets immediately after coming out of the cylinder may be pressed between dies and held compressed while the wax hardens sufficiently to retain the shape imparted by the dies.

In making some molded articles it is preferable to mix the fibrous constituents in a loose condition with melted Montan wax and thus produce a pulp which is subsequently molded under pressure to the desired shape, the material being allowed to cool in the mold sufficiently to cause the wax to set or harden and thus to retain the shape imparted by the molds to the pulp.

A molded stock produced in this manner, or the fiber board impregnated as above described, can be machined with entirely satisfactory results, the treated stock acting in this respect much like vulcanized fiber.

While, as above stated, we prefer to use Montan wax, both carnauba and candelilla waxes have properties very similar to those of Montan and can be substituted for it. However, they are considerably more expensive and both have a more pronounced tend-

ency than Montan to shrink or contract upon cooling.

Other waxes and even oils may be blended with Montan, and oil soluble coloring materials may be used with it. In making any of these blends or mixtures, however, care should be taken not to reduce the melting point, or more especially the softening point, of the mixture so far that the impregnating medium will be liable to ooze from the impregnated fiber board, or the surface thereof become sticky or tacky at high atmospheric temperatures, or those temperatures to which the material must reasonably be expected to be subjected while in use. For ordinary purposes it is reasonable to expect that treated fiber board may have to stand temperatures up to 130° or 140° F. when they are exposed to the sun. Montan wax will not soften at temperatures considerably above the latter figure, but in making any mixtures of this wax with oils, other waxes, or the like, it is desirable to bear these temperature requirements in mind. For special uses the temperature limits may vary considerably in either direction from those above mentioned. We prefer, however, to make any of these waxy impregnating compounds with at least a predominating percentage of Montan wax.

Some fiber boards include a very high percentage of fiber made from leather scrap, the percentage varying with the grade of the board. Usually a considerable percentage of wood pulp, rag stock, or both, are associated with the leather waste constituents, and in some boards these other ingredients predominate. The characteristics of fiber board of this character can be improved very substantially by the treatment above described, and the article or product resulting from such treatment is improved in substantially the same respects that have been described hereinbefore.

While we have herein disclosed preferred embodiments of our invention and preferred methods of practicing the process provided by this invention, it will be understood that this disclosure has been made rather by way of illustration than limitation, and that the invention is susceptible of embodiment in a considerable variety of forms and may be practiced in other ways than those specifically described without departing from the spirit or scope of the invention.

Having thus described our invention, what we desire to claim as new is:

1. That improvement in processes of treating fiber bodies which consist essentially of unvulcanized fiber, which consists in forcing air under pressure into the microscopic pores and cells of said body, subsequently, while holding said air under pressure in said pores and cells, forcing into said body a melted waxy material which remains hard

and brittle at high atmospheric temperatures but is sufficiently fluid at 250° F. to be forced into the pores and cells of the fiber body, then allowing the air imprisoned in said pores and cells to expand and thereby to eject a part of the impregnating medium, and later allowing said impregnated body to cool sufficiently to cause the waxy material to harden therein.

2. That improvement in processes of manufacturing fiber articles which consists in coating the fibrous constituents of the article and bonding the fibers thereof together substantially throughout the article with a melted waxy material which remains hard at all temperatures below 140° F., subsequently allowing the article so treated to cool sufficiently to solidify said waxy material, and mechanically confining said article while it cools to hold it in the desired shape until said waxy material has hardened.

3. That improvement in processes of treating fiber bodies of a porous character and consisting essentially of unvulcanized fiber, which consists in forcing into such a body substantially throughout the thickness thereof a melted waxy material which remains hard and non-tacky at high atmospheric temperatures, subsequently allowing said body to cool sufficiently to cause said material to harden, and mechanically confining said body while it cools to hold it in the desired shape until said material has hardened.

In testimony whereof we have signed our names to this specification.

ROGER W. CUTLER. 100  
JOSEPH R. COOLIDGE, III.

100

105

110

115

120

125

130